

W. VOLLMER & A. F. GIBBONEY.

INGOT MOLD.

APPLICATION FILED JUNE 17, 1912.

1,051,787.

Patented Jan. 28, 1913.



Fig. 1



Fig. 2.



Witnesses:-

Willard Burrows.

William F. Naes.

Inventors:-  
William Vollmer.  
Adolphus F. Gibboney.  
by their Attorneys:-  
Thomas & Ward

# UNITED STATES PATENT OFFICE.

WILLIAM VOLLMER AND ADOLPHUS F. GIBBONEY, OF BURNHAM, PENNSYLVANIA,  
ASSIGNORS TO THE STANDARD STEEL WORKS COMPANY, OF BURNHAM, PENN-  
SYLVANIA, A CORPORATION OF PENNSYLVANIA.

## INGOT-MOLD.

1,051,787.

Specification of Letters Patent. Patented Jan. 28, 1913.

Application filed June 17, 1912. Serial No. 704,195.

To all whom it may concern:

Be it known that we, WILLIAM VOLLMER and ADOLPHUS F. GIBBONEY, citizens of the United States, residing in Burnham, county 5 of Mifflin, State of Pennsylvania, have invented certain Improvements in Ingot-Molds, of which the following is a specification.

The object of our invention is to provide 10 means for casting steel ingots, so as to reduce that portion of the ingot which must be removed due to piping or unevenness. This object we attain in the following manner, reference being had to the accompanying 15 drawing, in which:—

Figure 1, is a vertical sectional view of an ingot mold illustrating our invention and showing the ingot in position; Fig. 2, is a plan view; and Fig. 3, is a sectional plan 20 view on the line 3—3, Fig. 1.

Referring to the drawings, A is the mold having a pouring opening either at the top or at the bottom. The pouring opening, in the present instance, is shown at the top. 25 A mold of this type is usually filled from the top or from the bottom. The upper end of the mold is recessed for the reception of a sand ring or core B and between the said ring and the body of the mold is a non-con-

ducting lining C of asbestos or magnesia. The internal diameter of the ring is preferably the same as the internal diameter of the mold, so that the upper portion of the ingot is not contracted when being poured. 30

35 D is a metallic plate, mounted upon the top of the ingot mold, having perforations  $d$  to allow the gases to escape as the ingot cools.

$i$  is a layer of black lead which is placed 40 upon the molten metal after it is poured, so as to retain the heat and yet allow the gases to pass off therethrough and through the perforations in the plate D. This layer of black lead is usually about an inch in thick- 45 ness.

The ring or core B is made of molding or core sand and as it is a poor conductor, it will allow the top of the molten ingot to retain its heat so that the metal will set with the least amount of piping. 50

The lining of asbestos or magnesia prevents the heat passing from the sand ring to the body of the mold and by covering the top of the ingot with black lead, this also assists in retaining the heat. Consequently, 55 the top of the mold cools very slowly and prevents piping.

The operation is as follows:—The mold is placed in position with the sand ring set in the recess in the upper part of the mold. 60 The molten metal is then poured into the mold, preferably from the top and, when the mold is filled to the proper height with the molten metal, the layer of black lead is then placed on the metal and the perforated 65 plate is placed in position upon the mold. The mold is then allowed to gradually cool and we find that as it cools a solid ingot is the result with, perhaps, a slight honey-combing at the upper surface, which can be 70 cut after the ingot is taken from the mold; the result being a solid ingot of superior quality.

We claim:—

The combination of an ingot mold having a recess at its upper end; a sand ring in the recess and an asbestos lining mounted between the ring and the inner wall of said recess; with a section of black lead placed in the ingot mold on top of the ingot and 80 within the sand ring.

In testimony whereof, we have signed our names to this specification, in the presence of two subscribing witnesses.

WILLIAM VOLLMER.  
ADOLPHUS F. GIBBONEY.

Witnesses:

W. M. H. WREN,  
W. E. MACK.